

## UNITED STATES PATENT OFFICE

2,184,956

## BLENDING AGENT FOR GASOLINE

Edwin R. Gilliland, Cambridge, Mass., and Raphael Rosen, Elizabeth, N. J., assignors to Standard Oil Development Company, a corporation of Delaware

No Drawing. Application February 6, 1937,  
Serial No. 124,468

9 Claims. (Cl. 44—9)

This invention relates to blending agents for gasoline to improve the anti-knock properties thereof and pertains more particularly to organic blending agents employed in relatively high concentrations in the gasoline.

The trend toward increasing the compression ratio of internal combustion motors in order to obtain greater efficiency has naturally increased the demands for motor fuel having higher anti-knock properties. The anti-knock properties of motor fuels is usually expressed in octane number, obtained by the method recommended by the Cooperative Fuel Research Committee of the Society of Automotive Engineers. According to this method an increase in octane number indicates an increase in anti-knock properties of the fuel.

Motor fuels produced by the common methods of refining do not have sufficiently high octane number to meet the requirements for high compression motors employed for aviation and automobiles. To meet this deficiency, it is a common practice to add an anti-knock agent such as tetraethyl lead or other metallo-organic compounds. The extent of improvement obtained by the addition of 1 cc. tetraethyl lead to gasoline is known as the lead susceptibility of the gasoline and varies with different types of gasoline.

Straight run gasoline of the same octane number derived from the various crude petroleum sources and cracked gasoline from different types of cracking processes have different lead susceptibilities. The reason why a measured quantity of tetraethyl lead does not have the same effect on all types of gasoline having the same octane number has not been definitely established. It has been found that as a general rule, subject to some exceptions, the higher the octane number of the gasoline the poorer the lead susceptibility. For this reason the octane number of high grade gasoline cannot be boosted to the same extent by the addition of 1 cc. of tetraethyl lead as can be obtained when added to a low grade gasoline. Moreover, a gasoline which has been improved by the addition of 1 cc. of tetraethyl lead is not improved to the same extent by the addition of a second cc. In other words, the improvement in octane number obtained by tetraethyl lead is not a linear function of its concentration. For these reasons the octane improvement which can be obtained by the addition of tetraethyl lead to the highest grade gasoline without forming objectionable lead deposits in the motor and introducing other operating difficulties, is limited. Moreover, in some

localities the use of tetraethyl lead or other lead alkyls is prohibited and in other localities restrictions are placed upon the concentration of lead.

Partly with the view of removing these limitations and partly to produce cheaper substitutes for tetraethyl lead and other metallo-organic compounds, intensive investigations have been made to discover other anti-knock blending agents which may be used in lieu of, or in addition to tetraethyl lead and other lead alkyl compounds.

More particularly, there is an urgent need for cheap blending agents which will impart an improvement in octane number which may be used in much greater concentrations than is desirable or permissible with respect to tetraethyl lead.

From previous investigations, it has been found that certain of the oxygenated hydrocarbons such as alcohols, ethers, ketones and aldehydes and particularly those having branched molecular structure improve the octane number when blended with gasoline. These compounds are not as potent as lead alkyls and are used in concentrations of entirely different order than when using leaded alkyl compounds. Whereas these organic blending agents are used in concentrations ranging from 10 to 50 or more percent, for example, tetraethyl lead is used in concentrations from .05 to .5 percent. In view of the necessity of using such large concentrations of anti-knock blending agents of this type, these agents must not only be capable of effecting a material improvement in the octane number of the gasoline when blended therewith, but they must have other properties comparable with that of the gasoline base. For example, in addition to improving the anti-knock properties, these blending agents must be volatile with the gasoline, miscible in large proportions with the gasoline, relatively insoluble in water, have a fuel value not materially lower than that of gasoline, and must not affect the functioning of other gasoline addition agents such as anti-oxidants and gum inhibitors. Furthermore, in order to impart maximum benefits to multi-cylinder motors, it is desirable to have the anti-knock agent vaporize with the constituents of the gasoline which have the lowest anti-knock properties. It is now known that because of fractional separation in the intake manifold of the motor each cylinder in a multi-cylinder motor does not obtain the same proportion of all constituents of the gasoline under all conditions of operation. For example, some cylinders may be charged

with a fuel which is relatively rich in higher boiling constituents and lean in lower boiling constituents. Other cylinders may be charged with fuel rich in intermediate constituents and 5 lean in high and low-boiling constituents, and other cylinders may be charged with fuel rich with low-boiling constituents and lean in higher boiling constituents. In order to prevent knocking in such motors the charge to each cylinder 10 should have high anti-knock properties.

It is generally known that the lower boiling fractions of gasoline have better anti-knock properties than the intermediate and higher boiling fractions. Consequently, for most effective results the anti-knock agent should vaporize with the intermediate and higher boiling fractions of the gasoline. Since tetraethyl lead vaporizes with the highest boiling fraction, it is most effective in reducing knock in the cylinders 15 20 pulling a charge rich in high-boiling and normally low anti-knock constituents and it is least effective for reducing knock in the cylinders pulling a charge rich in intermediate or low-boiling constituents. Since the low-boiling constituents 25 have relatively high anti-knock, it is particularly desirable that the anti-knock agent vaporize with the intermediate fractions of the gasoline. In addition to all these requirements for a satisfactory blending agent of this type, such agents 30 must be available in large quantities at relatively low cost somewhat comparable to gasoline.

Moreover, to meet requirements for extremely high octane number motor fuel for some types of aviation service metallo-organic anti-knock 35 agents have been added to the blend in order to get a further improvement in octane number. In other cases it is desirable to use lower concentrations of such blending agents and to supplement their use with tetraethyl lead because of the failure of such agents to satisfactorily meet all of the above requirements. In either case, it is important that the blended fuel have a good lead susceptibility. As already 40 pointed out, the lead susceptibility in general decreases as the octane number of base fuel increases and this generality, subject to some exceptions, applies to blended fuels as well as to unblended gasoline.

It has been found, however, that some blending 50 agents are not only capable of imparting an improvement in octane number, but the lead susceptibility of the resulting blend is much greater than would reasonably be expected from the octane number of the blend. Blending agents 55 of this character are of great value since they make possible the production of motor fuel having an octane value materially higher than could be obtained otherwise.

Our invention has for its object to provide a 60 blending agent which will satisfactorily meet the requirements above set forth.

More specific objects of our invention are to provide organic blending agents which are more 65 potent for improving the octane number of the gasoline and which when blended with gasoline will produce a blended motor fuel which has an extremely high lead susceptibility, much greater than would be expected from the octane number 70 of the blend.

Other specific objects of our invention will be apparent from the more detailed description 75 hereinafter.

As a result of our investigations we have dis- 76 covered that ethers boiling within the range of

gasoline or not materially higher, which have a branched chain structure, and which are formed from di- and tri-hydric alcohols are more potent in improving octane number, and produce a blend of better lead susceptibility than any of the straight chain compounds thus far investigated. We have also found that those having a branched chain containing a tertiary carbon atom are most effective. These compounds may be classified as glycol or glycerol ethers.

The glycol ethers may be expressed by the general formula  $R_1-O-R_2-O-R_3$ , where  $R_2$  is an alkylene radical having at least 2 carbon atoms,  $R_1$  is an alkyl radical,  $R_3$  is either hydrogen or an alkyl radical and  $R_1$ ,  $R_2$  or  $R_3$  is a branched group, preferably one having a tertiary or quaternary carbon atom. A tertiary carbon atom is one which is directly connected to three separate alkyl radicals and a quaternary carbon atom is one which is directly connected to four 20 separate alkyl radicals.

The glycerol ethers may be expressed by the general formula:



where  $R_2$  is an alkyl radical having at least 3 30 carbon atoms,  $R_1$  and  $R_3$  are the same as the first formula and  $R_4$  is either hydrogen or an alkyl radical.

The ethers of these classes which boil within, or not materially above the end point of the 35 gasoline, are the only ones adapted for use as anti-knock blending agents. Among the ethers thus far investigated, the mono- and di-tertiary ether of ethylene glycol have been found most effective. The octane number and lead susceptibility of the mono-tertiary butyl ether is shown in the following table:

Table 1

| Fuel                                                         | C. F. R. octane number |          |                |          |
|--------------------------------------------------------------|------------------------|----------|----------------|----------|
|                                                              | Blend                  |          | Blending value |          |
|                                                              | Clear                  | 1 cc. Pb | Clear          | 1 cc. Pb |
| Gasoline base.....                                           | 73.9                   | 82.9     | -----          | -----    |
| 25 percent mono-tertiary butyl ether of ethylene glycol..... | 86.8                   | 91.1     | 127            | 117      |

A blend containing 10% of the di-tertiary butyl ether of ethylene glycol was found to increase the octane number of 73.9 to 77.3 and to have a clear blending value of 114.

It will be noted that the addition of 25% mono-tertiary butyl ether of ethylene glycol improved the octane number 12.9 points (from 73.9 to 86.8) and that this can be further increased 4.3 points (86.8 to 91.1) by the addition of 1 cc. of tetraethyl lead. This shows exceptionally good lead susceptibility considering the extremely high octane number of the blend.

It will also be noted from the blending values given in the table, that it is possible to produce a fuel having an octane number in excess of 100 by either of these compounds.

Tests made on these same general class of compounds, but which do not have a branched chain structure have shown them to be definitely pro-

knock. The data obtained from these tests are shown in the following table:

Table 2

| 5                                            | 10   | 15   | Fuel  | Octane number C. F. R. |           |                |
|----------------------------------------------|------|------|-------|------------------------|-----------|----------------|
|                                              |      |      |       | Blend                  |           | Blending value |
|                                              |      |      |       | Clear                  | +1 cc. Pb |                |
| (1) Gasoline base                            | 74.3 |      |       |                        |           |                |
| (2) 25% mono ethyl ether of ethylene glycol  | 70.6 | 67.5 | 59.5  |                        |           |                |
| (3) 10% mono methyl ether of ethylene glycol | 71.0 |      |       |                        |           |                |
| 25% mono N-butyl ether of ethylene glycol    | 62.2 |      | 25.9  |                        |           |                |
| 25% mono butyl ether of diethylene glycol    | 48.7 |      | -28.1 |                        |           |                |

It will be apparent from these data that the addition of these unbranched compounds as distinguished from the branched compounds herein described actually induce knocking in the motor fuel.

Among other branched ethers of ethylene glycol which are particularly effective as anti-knock agents are the mono- and di-isopropyl ether, isopropyl tertiary butyl ether, methyl tertiary butyl ether, ethyl tertiary butyl, the branched mono- and di-amyl ethers, methyl, ethyl, propyl and isopropyl branched amyl ethers and the various branched butyl-amyl ethers. The corresponding ethers of propylene glycol and butylene glycol having boiling points within the desired range are likewise effective.

Among the effective glycerol ethers are the 1,2 di-methyl, tri-methyl, tri-ethyl and the 1,3 di-isopropyl.

These ethers may be readily prepared by refluxing the glycols or the glycerines with branched alcohols in the presence of a catalyst such as sulfuric acid. For example, mono- and tertiary butyl ether of ethylene glycol may be prepared by refluxing tertiary butyl alcohol with ethylene glycol in the presence of sulfuric acid. As a specific example, 800 cc. of tertiary butyl alcohol, 200 cc. of ethylene glycol and 36 cc. of 66° Bé. sulfuric acid were refluxed for one hour at 70° C. The mixture was then neutralized and fractionated giving 175 cc. of mono-tertiary butyl ether of ethylene glycol, 50 cc. of di-tertiary butyl ether of ethylene glycol and 75 cc. of unreacted glycol.

The blending agent may comprise any one of the branched ethers of di- and tri-hydric alcohols boiling below or not materially above the end point of gasoline or it may comprise any desired mixture of these compounds.

Another advantage of using this type of ethers as blending agents for gasoline is that certain of them, such as mono- and di-tertiary butyl ether of ethylene glycol boil in the intermediate range of gasoline and therefore are particularly effective for reducing knocking in cylinders fed with a charge rich in intermediate constituents. The mono-tertiary butyl ether boils at 302° F. and the di-tertiary at 336° F.

By the term "ether", as used in this description and in the claims, is signified compounds containing true ether groups, characterized by carbon atoms interlinked through an oxygen atom, with only a single oxygen atom joined directly to a carbon atom in an ether group.

Having described the preferred embodiment of our invention, it is understood that it embraces such other modifications and variations as come

within the spirit and scope thereof. It is also understood that it is not our intention to unnecessarily limit the invention or to dedicate any novel features thereof.

We claim:

1. A motor fuel for internal combustion motors comprising gasoline hydrocarbons blended with a branched ether of a polyhydric alcohol selected from the class consisting of glycols and glycerols in substantial amount sufficient to improve the anti-knock properties of the motor fuel, said ether boiling substantially within the gasoline boiling range and having only a single oxygen atom linked directly to a carbon atom in an ether group.

2. A motor fuel for internal combustion motors containing gasoline hydrocarbons and a tertiary ether of a polyhydric alcohol selected from the class consisting of glycols and glycerols, in a substantial portion sufficient to materially improve the anti-knock properties of the fuel, said ether boiling substantially within the gasoline boiling range and having only a single oxygen atom joined directly to a carbon atom in an ether group.

3. A motor fuel for internal combustion motors comprising gasoline hydrocarbons blended with a substantial quantity of a branched ether of a glycol to materially improve the anti-knock properties of the motor fuel, said ether boiling substantially within the gasoline boiling range and having only one oxygen atom linked directly to a carbon atom in an ether group.

4. A motor fuel for internal combustion in motors comprising gasoline hydrocarbons blended with a substantial amount of a tertiary ether of a glycol to materially improve the anti-knock properties of the motor fuel, said ether boiling substantially within the gasoline boiling range and having only a single oxygen atom attached directly to a carbon atom in an ether group.

5. A motor fuel for internal combustion motors comprising gasoline hydrocarbons blended with a substantial amount of a branched ether of a glycerol to materially improve the anti-knock properties of the motor fuel, said ether boiling substantially within the gasoline boiling range and having only one oxygen atom linked directly to a carbon atom in an ether group.

6. A motor fuel for internal combustion motors comprising gasoline hydrocarbons blended with a substantial amount of a tertiary ether of a glycerol to materially improve the anti-knock properties of the motor fuel, said ether boiling substantially within the gasoline boiling range and having only a single oxygen atom linked directly to a carbon atom in an ether linkage.

7. A motor fuel for internal combustion motors comprising gasoline hydrocarbons blended with a substantial quantity of a tertiary butyl ether of ethylene glycol to materially improve the anti-knock properties of the motor fuel.

8. A motor fuel for internal combustion motors comprising gasoline hydrocarbons blended with a substantial quantity of mono-tertiary butyl ether of ethylene glycol to materially improve the anti-knock properties of the motor fuel.

9. A motor fuel for internal combustion motors comprising gasoline hydrocarbons blended with a substantial amount of di-tertiary butyl ether of ethylene glycol to materially improve the anti-knock properties of the motor fuel.

EDWIN R. GILLILAND.  
RAPHAEL ROSEN.